

## UNITED STATES PATENT OFFICE

2,042,935

## CLEAN UP AGENT FOR VACUUM DEVICES

Daniel S. Gustin, Bloomfield, N. J., assignor to  
Westinghouse Lamp Company, a corporation of  
Pennsylvania

No Drawing. Application October 21, 1932,  
Serial No. 638,995

4 Claims. (Cl. 250—27.5)

This invention relates to the manufacture of vacuum devices and relates more particularly to the evacuation of incandescent electric lamps.

The practice of making incandescent electric lamps includes the operation of removing the gas from the bulb which is accomplished by the use of mechanical means such as vacuum pumps and in subsequently removing any residual gas by means of suitable substances termed "getters".

10 The present invention is directed to an improved form of getter or clean up agent to bring about a more complete clean up or removal of residual gas in vacuum devices such as incandescent electric lamps, radio tubes and the like. When 15 the term getter is used in the following specification and claims it is to be construed as a substance capable of reducing the greater portion or as near as possible all of the residual gas.

Many substances and combinations of substances have been employed as clean up agents 20 and one form of getter which has been successfully used contains 100 parts by weight of cryolite and 13 parts by weight of phosphorus.

When using such getter it is applied in the 25 form of a paste or liquid to the filament. When the filament is heated the getter is driven off. According to the accepted theory the cryolite is precipitated to the surface of the bulb and remains there to receive particles resulting from the 30 vaporization of the filament. The cryolite presents an irregular serrated surface so that the solid or opaque particles are widely distributed and become ineffective in obscuring the light or in other words the cryolite prevents blackening 35 of the bulb.

The phosphorus is in the form of red phosphorus which when heated is converted to yellow phosphorus in the form of a vapor. This vapor is ionized by the electric discharge between the lead 40 wires of the lamp or between the coils of the filament when such type of filament is employed. The ionization converts the yellow phosphorus vapor to red phosphorus which during conversion causes a physical chemical reaction with the 45 residual gas and removes the same in the sense that such gas is taken up by the red phosphorus particles which are widely distributed on the wall of the bulb and rendered invisible by reason of the cryolite which receives them.

I have found that the residual gas may be 50 completely removed or rendered ineffective if the ionization of the phosphorus or other vapor is increased by a more copious supply of electrons.

55 It is an object of the present invention, there-

fore, to provide a getter capable of promoting ionization.

Another object of the invention is to provide a getter containing a thermionically active material to promote the clean-up action of the getter. 5

Another object of the invention is to improve the vacuum in a sealed envelope by providing a substance for increasing the ionization of a vaporized constituent of a getter.

Other objects and advantages of the invention 10 will be apparent from the following description.

When practicing the present invention I have found that good results are obtained by using 15 getter composed of 100 parts by weight of cryolite and 13 parts by weight of phosphorus to which may be added 1.3% or less of a thermionically active substance such as barium carbonate. These substances may be thoroughly mixed with 20 a binder of nitrocellulose to provide a paste or it may be in liquid form so that the getter may be sprayed onto a filament. I have found that the barium oxide resulting from the heating increases 25 the electron emissivity and the carbon dioxide increases the amount of gas to be ionized. 25

It is to be understood that the present invention in its broadest aspects contemplates the use 30 of a material to increase the electron flow in the presence of a clean-up agent. Barium or other alkali earth metals may be used such, for example, as strontium, or the oxides or compounds of these substances may be used. Furthermore, the material for increasing or promoting ionization may be used with other getter materials in which ionization is effective to clean up residual 35 gases. As an alternative of the above getter composition I may use inorganic halogen compounds such as fluorids or double fluorids or sodium chlorid and similar halogen compounds. By adding to such getters a substance such as 40 barium or other substances to promote electron emission the resultant ionization improves the vacuum by the removal of the residual gas. 40

By reason of the present invention a clean-up 45 agent or getter is provided wherein the thermionically active material is a part of the mixture used. In the case of a cryolite phosphorus getter, for example, the cryolite performs its function as does the phosphorus while the added substance, by reason of the more copious supply 50 of electrons furnished, promotes ionization thus making the clean-up action more complete, resulting in a higher degree of vacuum than had heretofore been possible.

Although a preferred embodiment of the in- 55

- vention is shown and described herein it is to be understood that modifications may be made without departing from the spirit and scope of the invention as set forth in the appended claims.
5. What is claimed is:
1. In a vacuum device, a clean-up agent comprising phosphorus, cryolite and an alkali earth metal.
  2. In a vacuum device, a clean-up agent comprising phosphorus, cryolite and barium.
  3. A getter for a vacuum device comprising phosphorus and barium.
  4. A getter for a vacuum device comprising cryolite, phosphorus and barium.

DANIEL S. GUSTIN